

## UNITED STATES PATENT OFFICE

2,003,068

## PROTECTIVE FINISH

Michael J. Callahan, Parlin, N. J., assignor to  
E. I. du Pont de Nemours & Company, Wil-  
mington, Del., a corporation of Delaware

No Drawing. Application August 5, 1931,  
Serial No. 555,369

5 Claims. (Cl. 91—68)

This invention relates to a new two-system protective finish, more particularly it relates to a protective finish for automobile and metal surfaces in general comprising an undercoat which 5 contains pyroxylin and a top coat of polyhydric alcohol-polybasic acid resin which does not contain pyroxylin.

A large number of attempts have been made in the prior art to produce a satisfactory protective finish for the metal bodies of automobiles from various combinations of cellulose derivatives and polyhydric alcohol-polybasic acid resins. The prior practice has been concerned with either mixtures of the resin and pyroxylin, 10 or with systems in which the pyroxylin has been applied over a surfacer or a primer coating made from the resin. Insofar as I am aware a two system protective finish comprising a pyroxylin coating with a top coat of polyhydric alcohol- 15 polybasic acid resin as described herein is new and the advantages of this system for metal finishes has not been recognized.

This invention has as an object an improved protective finish for automobiles and other metal 20 surfaces. A further object resides in a new method of refinishing weathered pyroxylin surfaces, and particularly the weathered pyroxylin coatings of automobiles.

In the practice of the invention, the pyroxylin 25 or nitrocellulose coating may be designed as a primer, or the pyroxylin finish may be the usual built up primer-surfacer-pyroxylin enamel system. In either case a coating of a suitable clear or pigmented polyhydric alcohol-polybasic acid 30 resin is applied so as to produce a finishing system consisting of a pyroxylin coating surfaced with this type of resin.

For the resin top coat, I prefer to use a drying oil modified polyhydric alcohol-polybasic acid of 35 medium oil length. The following are examples of polyhydric alcohol-polybasic acid resins that are well adapted for the purposes of the present invention:

## Resin A

Parts by weight  
Glycerol ..... 17.11  
Linseed oil acids ..... 55.80  
Phthalic anhydride ..... 27.09

100.00

These ingredients are heated to 250° C. over a period of one hour and held at that temperature for five hours. The acid number of this 5 resin is 4 to 5.

## Resin B

|                      | Parts by weight |
|----------------------|-----------------|
| Glycerol             | 19.87           |
| Linseed oil acids    | 31.15           |
| China wood oil acids | 12.46           |
| Phthalic anhydride   | 36.52           |

5

These ingredients are heated to 225° C. over a period of one hour and held at that temperature for two and one-half hours. The acid number of this resin lies between 35 and 40. 10

## Resin C

|                    | Parts by weight |
|--------------------|-----------------|
| Glycerol           | 22.73           |
| Linseed oil acids  | 30.96           |
| Phthalic anhydride | 46.31           |

100.00

These ingredients are heated to 220° C. over a period of one and one-half hours and holding (two hours) at that temperature until an acid 20 number of 40-45 is obtained.

## Resin D

|                                          | Parts by weight |
|------------------------------------------|-----------------|
| Glycerol                                 | 28.43           |
| Cotton seed oil acids (double distilled) | 24.64           |
| Phthalic anhydride                       | 46.93           |

30

This mixture is heated to 225° C. over a period of one and one-half hours and holding (two hours) at that temperature until an acid number of 23-27 is obtained. 35

## Resin E

|                      | Parts by weight |
|----------------------|-----------------|
| Glycerol             | 22.73           |
| China wood oil acids | 30.96           |
| Phthalic anhydride   | 46.31           |

40

100.00

These ingredients are mixed in 33.3 parts by weight of "Hi-flash" naphtha and heated to the boiling point. The distillate, consisting of the naphtha and water of reaction, is condensed, collected and separated, the naphtha being returned to the reaction vessel. This cycle is allowed to continue and, after two and one-half hours heating, the clear reaction mixture has a temperature of 173° C. At this point 7.7 parts by weight of "Hi-flash" naphtha are added, and at 50 50 55

every one-half hour interval thereafter the same quantity is added as the resin content of the mixture increases until the end of seven hours when the cycle is allowed to continue for three 5 and one-half hours. The solid resin, acid number 55 to 60, may then be separated from the solution.

If an old pyroxylin surface is to be refinished, it is first cleaned. A fresh pyroxylin surface 10 may be finished with a coating of a resin of the type indicated as soon as the pyroxylin undercoat has dried. One or more coats of the clear or pigmented resin, dissolved in suitable solvents, is then applied directly, either by spraying or 15 brushing.

As a more specific illustration of the methods by which the invention may be carried out reference may be had to the following examples:

#### EXAMPLE I

20 A finishing system in which the resin coating is over a pyroxylin undercoat designed as a primer.

|                  | Parts by weight |
|------------------|-----------------|
| 25 Pigment       | 6.0             |
| Pyroxylin        | 4.0             |
| Plasticizer      | 2.0             |
| Drying oil       | 2.0             |
| 30 Resin "C"     | 5.8             |
| Toluol           | 20.7            |
| Ethanol (denat.) | 20.0            |
| Xylool           | 5.0             |
| Ethyl acetate    | 13.0            |
| 35 Butyl acetate | 21.5            |
|                  | 100.0           |

An enamel made from a polyhydric alcohol-poly-basic acid resin is applied over the above 40 priming coat by any well known method. A suitable enamel may be made up as follows:

|                                         | Parts by weight |
|-----------------------------------------|-----------------|
| Resin "A"                               | 61.3            |
| 45 Toluol                               | 28.2            |
| Carbon black                            | 7.9             |
| Drier solution (0.75% cobalt linoleate) | 2.6             |
|                                         | 100.0           |

50 Viscosity: 24.4 seconds in No. 10 cup.  
Total solids: 69.7%.

#### EXAMPLE II

A further illustration of the type of enamel 55 suitable for use over the above pyroxylin priming coat, I may use the following formulation:

|                                         | Parts by weight |
|-----------------------------------------|-----------------|
| Resin "B"                               | 28.8            |
| 60 Toluol                               | 52.2            |
| Chrome orange pigment                   | 18.4            |
| Drier solution (0.75% cobalt linoleate) | 0.6             |
|                                         | 100.0           |

65 Viscosity: 20 seconds in No. 10 cup.  
Total solids: 49.9%.

#### EXAMPLE III

Clear resin coating over a "built-up" pyroxylin 70 enamel

Frequently it is desirable to have the coloring material present in the pyroxylin undercoat instead of in the polyhydric alcohol-polybasic acid resin topcoat. In this case I prefer a built-

up finish as the undercoat, which consists of a primer, a surfacer and a pyroxylin enamel. The primer and surfacer may be of any well known composition which will provide good adhesion and produce a smooth surface, such as those of the oleoresinous type containing oils, driers, pigments, fillers, diluents, etc. The primer and surfacer are baked and sanded and a pyroxylin enamel of the following composition applied:

|                 | Parts by weight |
|-----------------|-----------------|
| Colored pigment | 9.0             |
| Pyroxylin       | 13.0            |
| Plasticizer     | 4.3             |
| Softener        | 2.8             |
| Ester gum       | 3.5             |
| Ethyl acetate   | 6.1             |
| Butyl acetate   | 23.9            |
| Butyl alcohol   | 6.0             |
| Ethyl alcohol   | 9.3             |
| Toluol          | 22.1            |
|                 | 100.0           |

A clear resin coating formulated as follows is applied directly over the above built-up system:

|                                         | Parts by weight |
|-----------------------------------------|-----------------|
| Resin "C"                               | 26.1            |
| Hi-flash naphtha                        | 73.1            |
| Drier solution (0.75% cobalt linoleate) | 0.8             |
|                                         | 100.0           |

#### EXAMPLE IV

Resin enamel over a "built-up" pyroxylin finish

|                                         | Parts by weight |
|-----------------------------------------|-----------------|
| Resin "D"                               | 20.7            |
| Hi-flash naphtha                        | 51.8            |
| Titanium oxide-barium sulfate pigment   | 26.9            |
| Drier solution (0.75% cobalt linoleate) | 0.6             |
|                                         | 100.0           |

Viscosity: 21 seconds in No. 10 cup.  
Total solids: 48.0%.

It is preferred to use a pigment of the same color in the pyroxylin enamel as in the resin topcoat, in this example, white.

An important application of the present invention is the refinishing of pyroxylin coatings on automobiles which have deteriorated through weathering. Pyroxylin enamels of the built-up 60 type, referred to in Examples III and IV, are known to be very useful in themselves as coating compositions, having unusual luster, flexibility, hardness, etc. The one main disadvantage of this type of coating is that outside exposure causes the film to chalk and dull. The refinishing of automobiles by the prior practice when these coatings finally weather and dull with age is, however, a costly undertaking inasmuch as a satisfactory job necessitates the removal of the old finish, the proper preparation of the metal, and the application of new coatings of the expensive nitrocellulose finish. I have discovered that the application to the old weathered pyroxylin finish of a clear or pig- 70 75

mented coating of polyhydric alcohol-polybasic acid resin as described herein imparts to the weathered coating a finish equally as lustrous and pleasing as the original pyroxylin finish with the added advantage of the improved durability and long lasting qualities contributed by this resinous surfacing. A particular advantage of my invention, therefore, is that I may refinish the metal surface so coated and dulled from weathering by applying a clear or pigmented polyhydric alcohol-polybasic acid resin directly over this weathered pyroxylin enamel.

In the application of the invention to the refinishing of weathered pyroxylin finishes of automobiles and of other metal surfaces, the old pyroxylin surface is thoroughly cleaned of all foreign material. This may be done with ordinary detergents such as a neutral soap. The old finish may be sanded, wet or dry, to prepare a smooth surface. A clear or pigmented polyhydric alcohol-polybasic acid resin, made in accordance with the foregoing examples of these resins or by any other suitable method, dissolved in suitable solvents is then applied directly, either by spraying or brushing. Two or more coats are frequently desirable.

#### EXAMPLE V

I have found the following system useful in the application of the invention for refinishing weathered pyroxylin finishes:

Pyroxylin undercoat: the built-up system of Example III, exposed to weathering.

#### Resin topcoat

|                                         | Parts by weight |
|-----------------------------------------|-----------------|
| Resin "B"                               | 28.8            |
| Toluol                                  | 52.2            |
| Ultramarine pigment                     | 18.4            |
| Drier solution (0.75% cobalt linoleate) | 0.6             |
|                                         | 100.0           |

Viscosity: 20.0 seconds in No. 10 cup.

Total solids: 49.9%

#### EXAMPLE VI

As a further illustration of the application of a polyhydric alcohol-polybasic acid resin enamel over a built-up pyroxylin finish which has been exposed to weathering, I may employ the following system:

Pyroxylin undercoat: the built-up system of Example III, exposed to weather.

#### Resin topcoat

|                                         | Parts by weight |
|-----------------------------------------|-----------------|
| Resin "E"                               | 27.3            |
| Chrome green pigment                    | 13.5            |
| Xylol                                   | 23.3            |
| Toluol                                  | 7.8             |
| Butyl acetate                           | 20.5            |
| Ethyl acetate                           | 3.6             |
| Butyl alcohol                           | 3.5             |
| Drier solution (0.75% cobalt linoleate) | 0.5             |
|                                         | 100.0           |

Viscosity: 20.0 seconds in No. 10 cup.

Total solids: 50.8%.

In preparing this enamel, the pigment is advantageously dispersed by grinding with a 40% solution of the resin in equal parts by xylene and butyl acetate.

Where the original finish is marred, or weathered to an unusual degree, I have found it desirable to spray over the old finish a coat of py-

roxylin primer followed by two coats of pyroxylin surfacer. After wet sanding, two coats of a pigmented resin enamel of the type described above were applied. While this procedure includes the application of pyroxylin coat over the original, the refinishing cost is, nevertheless, considerably cheaper than the prior practice which necessitates the removal of the old finish inasmuch as a second pyroxylin coat cannot, with satisfactory appearance, be applied directly over the original coat in the absence of the top resin coating as herein disclosed.

As will be understood to those skilled in the art, various changes may be made in the ingredients and methods recited for carrying out the invention. Driers, plasticizers, pigments, etc., may be incorporated into the resin top coat as desired, and the application of both the pyroxylin and resin top coat may involve any of the usual methods of application, such as spraying, brushing, air drying, baking, etc.

In addition to the fusion method, and the method of making the resins in an inert solvent as described, any of the other known methods for making these resins may be used. The oils themselves, as castor oil, may be incorporated into the resins instead of the oil acids. When the oils are used instead of the corresponding oil acids, it is preferable, however, to first heat the oil and glycerol together in the presence of litharge or other suitable catalyst, until the two phases merge into a single phase, and then heat the resulting mono- or di-glyceride, or mixture thereof, with the polybasic acid until resinification occurs. Various other oil acids, oils, or the mono- and di-glycerides of the oils, of the drying, semi-, and non-drying type, may be used as constituents for modifying the film-forming characteristics of the resin. These modified polyhydric alcohol-polybasic acid resins, whether prepared from the oils or oil acids, are for the purposes of the present invention referred to as oil modified polyhydric alcohol-polybasic acid resins. Various other modifying agents may be incorporated into the resin as desired. Among these may be mentioned natural resins and resin acids, as rosin, damar and Congo, monobasic acids, as benzoic and stearic, and monohydric alcohols, as cetyl and benzyl alcohol.

It is preferred to use phthalic anhydride as the polybasic acid and glycerol as the polyhydric alcohol in making the resins. The phthalic anhydride may, however, be replaced in whole or in part by other polybasic acids such as adipic, succinic, sebacic, maleic, itaconic, tartaric, citric, tricarballylic, dilactylic, thio-dilactylic, salicyl-acetic, chlorphthalic, diphenic, naphthalic, pyromellitic, etc. Similarly, the glycerol may be replaced with other polyhydric alcohols such as ethylene glycol and higher homologs, di-ethylene glycol and other polyglycols, polyglycerol, sorbitol, pentaerythritol, monoacetin, glycerol mono-alkyl ethers, etc.

It will be apparent from the foregoing that I have developed a new two-system protective finish for metal surfaces which finds extensive use in the arts when it is desired to combine the beauty of pyroxylin finishes with exceptional durability, and particularly when it is desired to refinish the weathered pyroxylin coatings of automobiles and impart thereto the appearance of the original finish, together with added durability, without incurring the expense that has been necessary heretofore. The top coat of the system described herein dries fast and is, in

this respect, comparable to a pyroxylin finish and is a marked improvement over the old oil type system. Another advantage resides in the superior build and hiding qualities of the top 5 coat of my improved protective system. An important advantage in the practice of my invention, and particularly in the refinishing of weathered pyroxylin coated automobiles, is the high initial lustre that is obtained without the 10 rubbing and polishing steps usually required by other types of finishes.

As many apparently widely different embodiment of this invention may be made without departing from the spirit and scope thereof, it 15 is to be understood that I do not limit myself to the specific embodiments thereof except as defined in the following claims.

I claim:

1. An article of manufacture having a metal 20 surface covered with a coating the film forming material of which consists predominately of nitrocellulose, and a top coat on the nitrocellulose coating of polyhydric alcohol-polybasic acid resin containing in chemically combined form the acid 25 radicals of fatty oil acid.

2. The article set forth in claim 1 in which said resin is a glycerol-naphthalate resin contain-

ing in chemically combined form the acid radicals of fatty oil acid.

3. An article of manufacture having a metal 5 surface covered with a primer coating, an intermediate coating over said primer coating, and a resinous top coat over said intermediate coating, the film forming material of the intermediate coating consisting predominately of nitrocellulose and the film forming material of the top coat being polyhydric alcohol-polybasic 10 acid resin containing in chemically combined form the acid radicals of fatty oil.

4. A process of refinishing coatings the film forming material of which consists predominately of nitrocellulose which comprises applying over the weathered nitrocellulose coating a coating of a solution of polyhydric alcohol-polybasic acid resin containing in chemically combined 15 form the acid radicals of fatty oil.

5. A process of refinishing coatings the film 20 forming material of which consists predominately of nitrocellulose which comprises applying over the weathered nitrocellulose coating a coating of pigmented solution of glyceryl phthalate resin containing in chemically combined form 25 the acid radicals of drying oil acid.

MICHAEL J. CALLAHAN.